

Patented July 28, 1925.

1,547,692

# UNITED STATES PATENT OFFICE.

EDWARD ROBERT SCHMID, OF VERONA, NEW JERSEY, ASSIGNOR TO WESTINGHOUSE LAMP COMPANY, A CORPORATION OF PENNSYLVANIA.

## PREVENTION OF COIL SLIPPAGE ON MANDRELS.

No Drawing.

Application filed August 18, 1923. Serial No. 658,185.

To all whom it may concern:

Be it known that I, EDWARD ROBERT SCHMID, a citizen of the United States, and a resident of Verona, in the county of Essex and State of New Jersey, have invented a new and useful Improvement in the Prevention of Coil Slippage on Mandrels, of which the following is a specification.

This invention relates to the winding of coils of tungsten wire or the like on mandrels and more particularly to the prevention of slippage of such coils on the mandrels, after they are cut to length for use as incandescent filaments in electric lamps or the like.

An object of my invention is the application of a solution to wire, after the same is wound on a mandrel, to act as an adhesive and temporarily affix the wound wire to its mandrel, so that wire and mandrel may both be cut to length without slippage therebetween.

Another object of my invention is the employment of an inorganic salt which is readily soluble in hot water and only slightly soluble in cold water, for application as a hot solution to coiled filament on a mandrel, for the purpose of preventing relative movement therebetween while cutting the filament and mandrel to length.

A further object of my invention is the preparation of filament coiled on a mandrel and prevented from slipping thereon by the application thereto of a hot solution of sodium tetraborate or its equivalent.

A still further object of my invention is the utilization of a thin film of borax or its equivalent, to cause filamentary material, which has been coiled on a mandrel, as is usual in the manufacture of incandescent filaments for gas-filled lamps, to temporarily adhere to the mandrel without slippage thereon, even while and after cutting into finished lengths.

Other objects and advantages of the invention will become apparent as the description proceeds.

In the manufacture of filaments for gas-filled incandescent electric lamps, it is usual to prepare the same in the form of helical coils, by winding around a wire mandrel, composed preferably of iron, brass or other metal, and annealing in place thereon. After the filament, which is preferably tungsten wire, is wound on the mandrel and

annealed in place, it is cut into sections, the length of each section depending on the size of the lamp for which it is to be used. Difficulty has been experienced from slippage of the tungsten coil along or off the mandrel while the same is being cut into sections of the desired length. This is undesirable in that it affects the accuracy with which the coiled filament is cut into sections.

Various expedients have been devised for eliminating this trouble, for example, if the mandrel with the filament wound thereon is annealed at a relatively high temperature, so that substantially all resiliency is removed from the wound filament, especially if the mandrel at the same time is slightly oxidized, there is not great danger of slippage thereon. However, it is desirable to perform the annealing operation at a relatively low temperature and another means for obviating slippage is disclosed in the co-pending application of Schule and Hunt, Serial No. 652,487, filed July 19, 1923, Method and apparatus for preventing slippage of coil wound mandrel, and assigned to the Westinghouse Lamp Company.

Said application discloses the roughening of the mandrel after the filament has been coiled or wound thereon by passing the same through a bath of nitric acid or equivalent material and then through an annealing furnace. This results in a roughening of the surface of the mandrel, which consequently tends to prevent slippage of the coiled filament thereon. The process disclosed is desirable and good results have been obtained by its use. However, there is no provision made for providing a substance with definite adhesive properties for holding the filament in place on the mandrel, the friction between the filament and the roughened mandrel being relied on for this purpose.

According to my invention, I provide a tightly-adhesive film of material, which is preferably applied to the coil on the mandrel immediately after the annealing operation, which serves to hold the filament in place thereon until the cutting operation has been completed and which makes it possible to anneal at a lower temperature than heretofore. There are numerous materials which could be used to form such a binding film, but a large number of them offer difficulties, in that they can only be removed with the expenditure of considerable time.

and effort, involve an extra operation and most are of the type which would cause trouble if their removal were not complete. I preferably use a material which is highly soluble in hot water and only slightly soluble in cold water, for example, an alkali borate and apply the same in the form of a hot, relatively-concentrated solution to the coiled filament on the mandrel, after the same has been annealed. As the coiled filament and mandrel cools, the supersaturation point of the solution will be reached and a firmly adherent coating will remain to hold the coil in place on the mandrel. The same may then be wound up, cut to the desired length or lengths, the mandrel removed and the coils treated in the usual manner.

My invention will be better understood by a specific description of a preferred embodiment thereof as follows, but it is to be understood that other materials than that mentioned may be used without departing from the spirit of my invention.

Sodium tetraborate or borax,  $Na_2B_4O_7 \cdot 10H_2O$ , has a high solubility in hot water and is only slightly soluble in cold water. A 50% hot solution of borax is therefore preferably prepared and coils of filament wound on a mandrel, passed through such a solution immediately after they have been passed through the annealer. As the wire cools, the supersaturation point of the borax film is reached, resulting in the deposit of a firmly-adherent coating of borax thereon, to hold the coil in place on the mandrel. This borax film is glass-like, relatively flexible and exerts no deleterious effect on a tungsten filament. After the application of the borax film to the coiled filament on the mandrel, the same may be wound up on a spool as usual and when desired, it may be cut into sections of proper lengths, which sections may have the portions of the mandrel therein removed in the usual manner, for example, by dissolving out in hydrochloric or sulphuric acid solutions. The sections of coiled filament, after removal of the mandrel therefrom, may then be cleaned by treatment in a caustic solution in the usual manner. The film of borax thereon comes off readily during the mandrel dissolving operation.

Undoubtedly, the same results might be obtained from other inorganic compounds, for example, potassium tetraborate which has a high solubility in hot water and a comparatively low one in cold water. Such a material should also form a flexible film which does not react with tungsten, which does not undergo changes when exposed to the atmosphere and which can be dissolved in hydrochloric or sulphuric acid solutions. Although I have described in detail, a preferred method of practicing my inven-

tion, it is to be understood that the same is merely illustrative and that modifications may occur to those skilled in the art within the spirit and scope of the appended claims.

What is claimed is:

1. The method of preventing metallic filament coiled on a mandrel from slipping thereon comprising applying a coating of adhesive material thereto. 70
2. The method of preventing filament coiled on a mandrel from slipping thereon comprising applying a solution of an inorganic adhesive material thereto. 75
3. The method of preventing filament coiled on a mandrel from slipping thereon comprising applying a hot solution of adhesive material thereto. 80
4. The method of preventing filament coiled on a mandrel from slipping thereon comprising applying a hot solution of an alkali borate thereto. 85
5. The method of preventing a metal filament coiled on a mandrel from slipping thereon, comprising applying a hot supersaturated solution of an alkali borate thereto, whereby a film of adhesive material sets thereon immediately upon cooling. 90
6. The method of preventing filament coiled on a mandrel from slipping thereon comprising passing the same through a hot solution of sodium tetraborate. 95
7. The method of preventing a metal filament coiled on the mandrel from slipping thereon, comprising passing the same through a hot supersaturated solution of sodium tetraborate, whereby an adhesive film forms immediately upon cooling after the filament is withdrawn from the solution. 100
8. The method of preventing the relative movement of a mandrel and a coil wound thereon which comprises depositing a material from solution on said coil and mandrel. 105
9. The method of preventing slippage between a filament and a mandrel on which it is coiled comprising temporarily cementing the filament to the mandrel by means of a flexible film of an inorganic soluble material. 110
10. The method of preventing slippage between a filament and a mandrel on which it is coiled comprising annealing the same and temporarily cementing the filament to the mandrel by means of a flexible film of an inorganic soluble material. 115
11. The method of preventing slippage between a filament and mandrel on which it is coiled, comprising annealing the same, whereby internal strains in the filament are reduced so that the tendency to unwind or slip is minimized, and passing said filament and mandrel through a hot supersaturated solution of an alkali borate, whereby a flexible cementing film forms immediately upon cooling when the filament is withdrawn from the solution. 120
- 125
- 130

12. A wire coiled on a mandrel and prevented from slipping thereon by a coating of adhesive material applied thereto.
13. A mandrel with a wire wound thereon and prevented from slipping thereon by the application of a solution of adhesive material thereto.
14. A mandrel wound with filamentary material temporarily fixed in place thereon by means of a solution of an alkali borate applied thereto.
15. A mandrel wound with metallic filamentary material and coated with a hot supersaturated solution of an alkali borate whereby an adhesive film, temporarily affixing the filamentary material in place on the mandrel, is immediately formed upon cooling.
16. A mandrel of iron wire or the like wound with refractory metal wire temporarily held in place by a solution of sodium tetraborate applied thereto.
17. Refractory metal wire wound on a mandrel of iron wire or the like and treated with a hot supersaturated solution of sodium
- tetraborate to temporarily hold the wire in place on the mandrel.
18. An iron wire mandrel or the like to which a coil of tungsten wire is temporarily affixed and prevented from slipping thereon by means of a hot solution of sodium tetraborate, whereby the same may be cut into sections without relative displacement between the mandrel and the filament. 30
19. A metal mandrel wound with tungsten wire or the like, annealed and slippage between the wire and mandrel prevented by a film of an alkali borate applied thereto. 35
20. A readily soluble metal mandrel wound with tungsten wire or the like, annealed and coated with a hot supersaturated solution of an alkali borate, whereby slippage between the wire and mandrel is prevented by the formation of a film of adhesive material. 40
- 45

In testimony whereof, I have hereunto subscribed my name this 17th day of August, 1923.

EDWARD ROBERT SCHMID.